

Sept. 9, 1941.

P. L. SALZBERG

2,255,600

BLASTING INITIATOR

Filed Aug. 3, 1938



*Paul L. Salzberg*  
INVENTOR

BY *Thos. A. Wilson*  
ATTORNEY

## UNITED STATES PATENT OFFICE

2,255,600

## BLASTING INITIATOR

Paul Lawrence Salzberg, Carrcroft, Del., assignor  
to E. I. du Pont de Nemours & Company, Wil-  
mington, Del., a corporation of Delaware

Application August 3, 1938, Serial No. 222,835

15 Claims. (Cl. 102—9)

The present invention relates to new and improved blasting initiators and more particularly to an improved shell for the same.

As is well known in the art of blasting initiator manufacture, it has been necessary to avoid the use of certain types of shells in combination with particular classes of explosive compounds, due to the recognized incompatibility of said shell materials with charges containing said explosive compounds. In particular, certain explosive compounds react with shell materials to form dangerously sensitive substances. For example, shells containing copper are incompatible with explosive charges containing azides, especially lead azide. This is believed to be due to the reaction of copper with lead azide to form the dangerously sensitive copper azide. At any rate it is particularly disadvantageous that the highly desirable standard gilding metal shell, a copper-zinc alloy of high copper content, has never been successfully employed in conjunction with charges containing lead azide.

The object of this invention is a new and improved blasting initiator. A further object is a blasting initiator shell compatible with certain reactive explosive charges. An additional object is a blasting initiator provided with a shell of a metal not ordinarily compatible with lead azide, which shell has been treated to render it compatible therewith. Another object is a safe and improved initiator comprising a copper-containing shell in combination with a charge of lead azide. Other objects will be apparent from the following description of my invention.

I have found that the foregoing objects are accomplished by treating a copper-containing metal shell with a mercaptan or an organic composition having a mercaptan group. The shell thus treated may be employed in the manufacture of a safe blasting initiator containing explosive charges not compatible with copper, for example, lead azide. According to my invention, the entire surface of the blasting cap shell is exposed to the action of the mercaptan, whereby a protective coating results. This protective coating affords complete and uniform coverage, and has no tendency to become displaced.

Although mercaptans in general produce a desirable coating for metal shells, I prefer to use those characterized by a long-chain structure, as, for example, lauryl mercaptan (1-dodecanethiol), octyl mercaptan, or cetyl mercaptan (1-hexadecanethiol). These longer-chain compounds produce a film of superior quality.

According to one theory at least, the mercap-

5 tans combine chemically with the copper present in the shell, the reactive end of the mercaptan structure attaching itself to the metal surface, leaving a non-reactive film, the thickness of which is proportional to the length of the chain. This is believed to prevent formation of the highly sensitive azide which is considered to be formed ordinarily by the reaction between moisture, lead azide and copper, supposedly 10 through the hydrolysis of the azide and hydrazoic acid and further reaction of the latter with the copper. It is sufficient that copper shells treated with the mercaptan, according to my invention, are entirely satisfactory when employed with charges containing lead azide.

In carrying out my invention, my protective coat-forming composition, as hereinbefore mentioned, is added to such quantity of solvent that a solution of the desired concentration results. This solution may be applied to the blasting cap shell according to any of the commonly known methods for the application of protective coatings.

One method which requires only a short time, 25 but which has proved effective, is the tumbling barrel method of treatment. The shells to be treated are first cleaned in order to remove any film which might retard or prevent the action of the mercaptan. The cleaning agents employed are those in common usage for such purposes, for example, solvents such as acetone, alcohol, etc., or certain dilute mineral acids. After cleaning and drying, the shells are rumbled in a barrel containing a solution of the mercaptan 30 in a suitable solvent.

The following examples are given in order to illustrate this preferred method of operation.

## Example I

40 A 5% solution of lauryl mercaptan in benzene was introduced into a tumbling barrel. Blasting cap shells of gilding metal were then added, and the barrel rumbled for one hour. At the end of this period the shells were removed, the excess liquid drained, and the remaining liquid permitted to evaporate. When dry, the shells 45 were characterized by a film-like coating non-reactive with respect to hydrazoic acid.

## Example II

50 Separate solutions of lauryl mercaptan, octyl mercaptan and mercaptobenzothiazole were employed to coat numerous gilding metal shells. The lauryl mercaptan and octyl mercaptan were dissolved in benzene to form 5% solutions, where- as the mercaptobenzothiazole was in the form of

a 2.2% by weight acetone solution. In each instance, the tumbling barrel method was employed, the treatment extending over a one hour period. In order to evaluate the various mercaptans as coating agents, these treated shells were tested under identical conditions, together with untreated shells. The stability tests comprised loading both the treated and untreated shells with similar explosive compositions, including lead azide, and subjecting the loaded shells to an atmosphere of approximately 100% humidity. The shells were inspected at regular intervals, tests being made in order to detect the presence of copper azide. The results obtained are shown in the following tabulation.

5

copper-tin, for example. Furthermore, although my invention has been described particularly with respect to lead azide, it is understood that the general concept will be applicable to any shell material with respect to any initiator charge when neither is detrimentally reactive with mercaptan, where incompatibility otherwise would exist between said charge and said shell material. I intend, therefore, to be limited only 10 in accordance with the following claims.

I claim:

1. A blasting initiator comprising a mercaptan-treated metal shell, and in said shell an explosive charge incompatible with said metal.
2. A blasting initiator comprising a mercap-

15

| Storage period | Mercapto-benzothiazole treated shells | Octyl mercaptan treated shells | Lauryl mercaptan treated shells | Untreated shells |
|----------------|---------------------------------------|--------------------------------|---------------------------------|------------------|
| 1 month        | Negative test                         | Negative test                  | Negative test                   | Negative test.   |
| 2 months       | do                                    | do                             | do                              | Positive test.   |
| 3 months       | do                                    | do                             | do                              |                  |
| 4 months       | do                                    | do                             | do                              |                  |
| 5 months       | do                                    | do                             | do                              |                  |
| 6 months       | do                                    | do                             | do                              |                  |
| 7 months       | do                                    | do                             | do                              |                  |
| 8 months       | do                                    | do                             | do                              |                  |

The accelerated tests set forth in the foregoing table show that copper azide had formed on the untreated shells at the end of the second month, whereas the shells coated with the various mercaptans remained unaffected over a period of eight months.

The various mercaptans described hereinbefore are given merely as specific embodiments and should not be construed as limiting my invention. Other mercaptans having a long chain structure have been found equally desirable, cetyl mercaptan, for example.

The invention may be understood more readily by referring to the drawing which is a view of a blasting initiator shell provided with a coating of mercaptan, as described by the legends.

My invention, therefore, discloses an initiator that is new to the art, together with a process for making the same. The process employed for treating the initiator shell is characterized by simplicity and ease of application of the coating material. The adoption of the novel initiator permits the use of lead azide, as an explosive charge, particularly in any blasting caps, ordinary fuse-type or electrical, which are not moisture-proof, without necessitating an initiator shell free from copper. On the contrary, the lead azide may be charged directly into the treated copper-containing shell without danger that sensitive compounds will be formed. In addition, the mercaptan-treated copper shells are more resistant to corrosion than untreated shells.

From the foregoing description of my invention, it is apparent that many variations may be made without departing from the spirit and scope thereof. Although the discussion has been directed particularly toward gilding metal because this metal has been commonly employed, yet my invention is not limited to said gilding metal, but is applicable when any shell having a significant copper content is employed, as alloys of

30 tan-treated, copper-containing shell and in said shell an explosive charge incompatible with copper.

35 3. A blasting cap comprising an explosive charge including lead azide in a mercaptan-treated, copper-containing cap shell.

40 4. The blasting cap of claim 3, wherein the mercaptan employed is octyl mercaptan.

5. The blasting cap of claim 3, wherein the mercaptan employed is 1-hexadecanethiol.

6. The blasting cap of claim 3, wherein the mercaptan employed is mercaptobenzothiazole.

45 7. A blasting cap of the fuse-type containing an explosive charge comprising lead azide, said charge being contained in a mercaptan-treated, copper alloy cap shell.

8. A fuse-type blasting cap comprising a mercaptan-treated, copper-containing shell.

50 9. A process for treating copper-containing initiator shells, which process comprises subjecting said shells to the action of a solution consisting substantially of a long chain mercaptan.

10. The process of claim 9, wherein the mercaptan comprises 1-hexadecanethiol.

11. The process of claim 9, wherein the mercaptan comprises octyl mercaptan.

12. The process of claim 9, wherein the mercaptan comprises mercaptobenzothiazole.

55 13. A process for coating copper-containing initiator shells, which process comprises agitating said shells in a solution containing a mercaptan, draining off said solution, and drying the mercaptan-coated initiator shells.

60 14. A blasting initiator comprising an explosive charge enclosed in a mercaptan-treated, copper-containing cap shell.

65 15. A blasting initiator comprising an explosive charge including lead azide enclosed in a mercaptan-treated, copper-containing cap shell.

PAUL LAWRENCE SALZBERG.